

## UNITED STATES PATENT OFFICE

2,028,296

## METHOD OF REMOVING WATER OF GELATION

Milton J. Shoemaker, Madison, Wis., assignor, by mesne assignments, to Carbide and Carbon Chemicals Corporation, New York, N. Y., a corporation of New York

No Drawing. Application November 24, 1931,  
Serial No. 577,159

7 Claims. (Cl. 18—57)

This invention relates to a method for removing water rapidly and efficiently by a freezing process from solid cellulosic products which have been coagulated, regenerated or otherwise deposited from aqueous solutions and especially from such products as freshly formed sheets of regenerated cellulose (as from viscose) and of aliphil hydroxy-ethers of cellulose such as ethyl hydroxy-ethers which have a limited solubility 5 in caustic alkalies and to the product resulting therefrom.

Some of the objects of this invention are to cheapen the cost of drying films, threads or the like, of cellulosic products which have been 10 formed from water or water solutions, to cut the cost of the machinery necessary for drying, to simplify the drying operation by decreasing the shrinkage on drying, and to increase the strength of the material.

At the present time films of regenerated cellulose are made by coagulating a film of viscose in an acidified bath after which the film is led through a number of treating and washing baths. When the film is a continuous sheet, it finally 20 passes over a series of heated drums to dry the product to the desired moisture content. This latter operation must be carried out carefully on equipment which ordinarily is expensive, to produce a smooth, highly transparent, and lustrous article, such as is demanded by the trade. The evaporating costs are high since the wet sheet enters the drying machine with a water content of 75% to 90% (if no emollient is used) and this water must be practically entirely removed. If sheets of certain derivatives of cellulose, such as the hydroxy-ethers as previously 30 described, are made; approximately the same conditions obtain. During the evaporation of this large amount of water the sheet, if allowed to contract freely, is subject to excessive shrinkage, the average lineal shrinkage being about 30 to 35 per cent. This complicates the drying problems. However, when a sheet is dried on continuous machines it is kept under tension so that 40 there is little or no lineal shrinkage but there is some cross shrinkage. As a result the sheet is stretched, usually more or less unevenly, and there is considerable variation in the thickness and in the strength of the sheet both across and 45 in the machine direction. By my invention it is possible to eliminate over 50 per cent of the evaporation cost and machinery for making a continuous sheet and simultaneously cut the tendency to shrink during drying to a minimum. This lessened tendency to shrink greatly de-

creases the stretch in the dried sheet and makes for more uniformity in thickness and in the strength of the sheet both across and in the machine direction. In addition it is not necessary to handle, on the driers, the very tender film 5 having a high water content.

When the before mentioned cellulosic products are coagulated from a water solution, and after being further treated and/or washed to remove impurities in the form of other products of reaction and coagulating acids and salts, the coagulated material contains from 75% to 90% of water. This water may be described as water of gelation. All of this water of gelation, however, apparently is not held in the same way by the 10 coagulated cellulosic material. If about 55% to 60% of the water present in this coagulated material (containing about 75% to 90% of water) is removed, water will not again reenter appreciably the partially dehydrated film (containing 60% to 70% of water) even on prolonged soaking in water. The balance of the 20 water may be removed by drying but the dried material will again take up a like amount of water (60% to 70% of water) if soaked in 25 water. The first dehydration or de-gelation, therefore, is an irreversible phenomenon and I have called the water which is removed in this step non-reentrant water of gelation since such water cannot again enter the material after being 30 removed therefrom.

I have found that it is possible to remove the non-reentrant water of gelation by a freezing operation. If the freshly coagulated and washed material, for example, in the form of a film, is 35 frozen and then thawed, water drains from the surface thereof. About 55% to 60% of the water content of the film is removed by this procedure. The lineal shrinkage during this operation is about 6% for the hydroxy-ether. The presence 40 of an emollient such as glycerine reduces this shrinkage. The balance of the drying may be accomplished in the usual way, the additional shrinkage being about 8%. After the film is frozen and thawed, and the non-reentrant water 45 removed as by draining, the strength of the film is increased considerably over that of the initially coagulated film and its thickness is reduced. An emollient such as glycerine, is preferably introduced into the film after the non-re- 50 entant water has been removed. The film is run through the necessary bath of emollient in the usual manner.

The freezing operation may be carried out by placing the film against a cold surface or sub- 55

jecting it to cold air or to any suitable cold liquid. The film, if it is to be frozen in the air or any other gaseous fluid, is subjected to such gas cooled to a temperature below the freezing point of water. The rate of freezing depends upon the temperature and circulation of the air. If the gas circulates rapidly it freezes the film more rapidly, but it also causes cloudiness and for most purposes this is objectionable.

An excellent freezing method is that in which the coagulated cellulosic material is immersed in a liquid bath which is held at a temperature below the freezing point of water. Obviously the bath should be of such a material that it does not affect the film chemically. Mercury is especially suitable. Although various organic liquids such as toluene, gasoline, alcohols, carbon tetrachloride, acetone, etc., may be used, these liquids have the disadvantage of clouding the film too readily. Water solutions of salts in sufficient quantity which permit the solution to be cooled considerably below the freezing point of water may be used to advantage since the films frozen therein remain clear and bright. Solutions of ordinary salt (sodium chloride) or calcium chloride are suitable. The bath is cooled to a temperature from 5 to 15 degrees centigrade below the freezing point of water and the coagulated and washed film immersed therein. The ordinary film freezes quickly, ice forming a coating over the surface and extending through it in 10 to 20 seconds. The film may now be removed from the cold bath to a warmer place, to allow the ice to melt, or the film may be allowed to remain in the bath for a longer period of time. If the frozen film remains in a refrigerating bath of a solution of a salt in water for a period of time the ice again melts and the water resulting therefrom gradually diffuses into the refrigerating solution so that the film then may be removed with the ice completely liquefied. After the film has been defrosted and the excess water removed from the surface it may be dried in the usual manner. Thus the water may be removed by the diffusive action of a salt solution and water in the frozen state. This is liquefaction of the ice by a process other than melting, and at a temperature below the freezing point. Of course it is not necessary that the diffusive process involve the particular liquid in which the ice is formed. Other materials, such as a different liquid or solution may be used.

In another method a long length of the wet film is rolled onto a spool and this spool of film is then refrigerated at a suitable temperature as given above. This refrigeration may be carried out by keeping the spool in an ordinary refrigerating chamber, the exterior surface of the spool being subjected to the chilled air. It is advisable sometimes to wrap the spool in paper or like material to prevent too rapid circulation of air. After the entire spool is frozen it is again subjected to higher temperatures to thaw the ice that has been formed. After draining the excess water from the spool the wet film is then dried in the usual way.

Although my improved process has been described in connection with films it may be applied in like manner to filaments and other forms of cellulosic materials coagulated from a water solution thereof.

Moist films from which the reentrant water of gelation has been removed by my freezing process and which shrink but a small amount on drying may be used under certain conditions for

wrapping articles, bottle tops and the like. Such films are desirable and preferred over the freshly coagulated film where it is necessary to have a film that is less tender, which dries more quickly and where the tautness resulting from excessive shrinkage is not desirable.

From the foregoing disclosure it is apparent that the effective part of the process is the freezing. The conversion of the non-reentrant portion of the water of gelation from water of gelation to non-reentrant water apparently takes place by conversion of that portion, from water of gelation to frozen non-reentrant water. The removal of the frozen non-reentrant water is not necessarily practiced by melting, and may be carried out in numerous ways. Removal has been described by melting it, and also by dissolving it, as it were, by the diffusive or other definitive action of liquids thereon which are effective below the melting point of the ice, such as a salt solution in which the ice may be formed. Other known methods of removing ice may be applied, such as evaporation of the ice without melting it.

It is also to be understood that the invention may be practiced on materials from which part of the water has already been dried, but in which a portion of the non-reentrant water yet remains. In commercial practice of the invention, the methods employed for storing, conveying, or exposing the material after coagulation, and before freezing may be intentionally or inadvertently conducive to drying, and may effect partial drying. Such practice does not in any way mitigate the advantages of the present invention nor depart therefrom.

While cellulose regenerated from viscose, and the hydroxy ethers of cellulose have been specifically described, it will be understood that the functional property of hydration upon coagulation from water is common to cellulose and its derivatives, including the hydroxy ethers, and that part of the water so included by gelation is non-reentrant water. The present invention contemplates all such materials which are characterized by this property.

It will be understood that numerous changes in and departures from the processes particularly disclosed herein may be made without departing from the spirit and scope of the invention as expressed in the appended claims.

I claim:

1. The method of substantially decreasing the water content of a cellulosic film which has been coagulated from aqueous solution and which contains non-reentrant water of gelation, which comprises immersing said film in an aqueous refrigerating solution of a salt which is at a temperature below the freezing point of water, keeping said film in said liquid until said non-reentrant water of gelation freezes and diffuses into said refrigerating solution.

2. The method of drying a cellulosic product which has been coagulated from aqueous solution and which contains non-reentrant water of gelation, which comprises immersing said product in an aqueous refrigerating solution of a salt which is at a temperature below the freezing point of water, keeping said product in said liquid until said non-reentrant water of gelation freezes and diffuses into said refrigerating solution, removing said product from said liquid, and drying the moist product.

3. The method of substantially decreasing the water content of a cellulosic product which has

been coagulated from aqueous solution and which contains non-reentrant water of gelation, which comprises freezing said coagulation product in a solution, and removing the ice formed by said freezing process by the results of diffusion between the solution and the product containing the ice crystals at a temperature which is below the freezing point of said ice.

4. As a new article of manufacture, a water-moist film of a hydrated cellulosic product from which non-reentrant water of gelation has been removed, said film being characterized by uniform tensile strength in right-angular directions in the film.

10 5. As a new article of manufacture, a water-moist film of a hydrated cellulosic product from which non-reentrant water of gelation has been

removed, said film being characterized by uniform shrinkage and tensile strength in right-angular directions in the film.

6. As a new article of manufacture, a water-moist film of regenerated cellulose from which non-reentrant water of gelation has been removed, said film being characterized by the property of uniform shrinkage and tensile strength in right angular directions in the film.

7. As a new article of manufacture, a water-  
moist film of aliphil-hydroxy ether of cellulose  
from which non-reentrant water of gelation has  
been removed, said film being characterized by  
the property of uniform shrinkage and tensile  
strength in right angular directions in the film.

MILTON J. SHOEMAKER.